

# UNITED STATES PATENT OFFICE.

ANDREW J. BISHOP, OF ST. PAUL, MINNESOTA.

## COMPOSITION OF MATTER FOR FILLING TIRES.

1,099,336.

Specification of Letters Patent.

Patented June 9, 1914.

No Drawing.

Application filed November 4, 1912. Serial No. 729,308.

*To all whom it may concern:*

Be it known that I, ANDREW J. BISHOP, a citizen of the United States, residing at St. Paul, in the county of Ramsey and State 5 of Minnesota, have invented a new and useful Composition of Matter for Filling Tires, of which the following is a specification.

My composition consists of the following ingredients combined in substantially the 10 following proportions, viz.: Glue, about thirty-two pounds; glycerin, about fifty-one pounds; raw linseed oil, about eight pounds; molasses, about eight pounds; and pulverized or ground cork, about one pound.

15 In the preparation of the improved filler the glue is first dissolved in water, and then put with all the other ingredients into a pot or kettle, where the mixture is boiled until the water which has been added to dissolve 20 the glue has been boiled out. The ingredients thereby become thoroughly commingled, and when allowed to cool will set into a coherent, pliable, resilient, solid, mass.

In use, the mixture can be injected into a 25 tubular tire while still hot and fluid, so that it will set within the tire, or, if it is to be used with a tire which is open, such as the casing for double tube tires, it can be first molded or cast into a cylinder, and then 30 placed within the casing. When it is injected hot, it will expand slightly in cooling, so as completely to fill the tube. In either case the mixture will form a resilient, pliable non-inflammable, and non-combustible solid

filler which will make the tire independent 35 of punctures and which will avoid the trouble attendant upon the blowing out of air inflated tubes. The filler thus formed will form a coherent, elastic and pliable cushion. The glue forms the body of the 40 cushion and gives it coherence and strength, but if used alone it will harden and become brittle in use. I therefore use molasses and glycerin to make and keep it elastic and pliable, and add the linseed oil to prevent the 45 molasses from sugaring. I use pulverized or ground cork as one of the ingredients, in order to lighten the weight of the filler.

It is to be understood that the proportions specified are those which I have found to 50 produce the best results, but these proportions can be slightly varied without materially altering the character or quality of the filler.

I claim as my invention:

The herein described composition of matter for filling tubular tires, consisting of a cooked mixture of glue about thirty-two pounds, glycerin about fifty-one pounds, raw linseed oil about eight pounds, molasses 60 about eight pounds, and pulverized cork about one pound.

In testimony whereof I affix my signature in presence of two witnesses.

ANDREW J. BISHOP.

Witnesses:

ARTHUR P. LOTHROP,  
H. SWANSON.